

United States Patent [19]  
Koch

[11] 3,915,815  
[45] Oct. 28, 1975

[54] **ALKALINE ZINC ELECTROPLATING BATH**

[76] Inventor: **Reinhard Koch**, 6081 Geinsheim,  
Germany

[22] Filed: **Nov. 14, 1973**

[21] Appl. No.: **415,757**

[30] **Foreign Application Priority Data**

Nov. 15, 1972 Germany..... 2256000

[52] **U.S. Cl..... 204/55 Y; 260/29.2 EP; 260/72 R**

[51] **Int. Cl.<sup>2</sup>..... C25D 3/24**

[58] **Field of Search..... 204/55 Y, 55 R, 432, 44**

[56] **References Cited**

UNITED STATES PATENTS

|           |         |                    |            |
|-----------|---------|--------------------|------------|
| 2,288,318 | 6/1942  | Hoffman.....       | 204/55 Y   |
| 2,680,712 | 6/1954  | Diggin et al. .... | 204/55 Y   |
| 2,791,554 | 5/1957  | Winters.....       | 204/55 Y   |
| 2,860,089 | 11/1958 | Jackson .....      | 204/55 Y   |
| 3,227,638 | 1/1966  | Burnson.....       | 204/55 Y X |

|           |         |                |          |
|-----------|---------|----------------|----------|
| 3,472,743 | 10/1969 | Rushmere ..... | 204/55 Y |
| 3,655,534 | 4/1972  | Kampe .....    | 204/55 R |
| 3,806,431 | 4/1974  | Koch.....      | 204/55 Y |

*Primary Examiner—G. L. Kaplan  
Attorney, Agent, or Firm—Erich M. H. Radde*

[57] **ABSTRACT**

The alkaline zinc electroplating bath of the present invention contains as brightening agent the reaction product of

- a. polyethylene imine or polypropylene imine with
- b. an aromatic aldehyde,
- c. ammonia and/or ethylenediamine, or diethylene triamine and
- d. epichlorohydrin.

Due to the addition of said reaction product its cyanide content can be considerably reduced without impairing the brightness of the zinc deposit.

**9 Claims, No Drawings**

## ALKALINE ZINC ELECTROPLATING BATH

## BACKGROUND OF THE INVENTION

1. Field of the Invention bath and more particularly to a The present invention relates to a cyanide-containing zinc electroplating bath cyanide-containing zinc electroplating bath yielding smooth and bright to fully bright zinc plates, to a process of producing said baths, and to a method of using such baths for electroplating.

## 2. Description of the Prior Art

Cyanide-containing zinc baths for electrolytic deposition of zinc plates are known. Bright zinc plates of excellent throwing power, metal distribution, and brilliance are produced, when using such baths.

Cyanide-containing zinc baths require the addition of special brightening additives in order to produce zinc layers of high brilliance. Such additives are, for instance, amino-aldehyde derivatives such as aldehyde-alkanolamines, water-soluble polyvinyl alcohols, salts of metals of the groups VIIB or VIII of the Periodic System, and sugars. The amounts of such additives, however, must be carefully adjusted in relation to the zinc content and/or the cyanide content of the bath.

More recently, and in ever increasing numbers, weakly acid or alkaline cyanide-free zinc baths or baths of a low cyanide content are used in order to meet the requirements of pollution control which demands special waste disposal treatment and equipment so as to conform with legal provisions. However such cyanide-free zinc baths or baths of a low cyanide content usually do not yield zinc coating of a brilliance comparable to that attained with cyanide-containing zinc baths.

## SUMMARY OF THE INVENTION

It is one object of the present invention to provide a novel and advantageous cyanide-containing zinc bath and especially a zinc bath of a low cyanide content which yields bright zinc coatings, has a satisfactory throwing power, and achieves good metal distribution, said bath exhibiting the properties of a good zinc bath of the usual high cyanide content, said bath permitting to considerably decrease its cyanide content even when operating at a current density below 1 amp./sq.dm.

Another object of the present invention is to provide a simple and effective process of producing such a zinc bath.

A further object of the present invention is to use such a zinc bath for zinc electroplating and the deposition of a bright zinc coating.

Other objects of the present invention and advantageous features thereof will become apparent as the description proceeds.

In principle the bright zinc plating bath according to the present invention contains, in addition to an alkali metal hydroxide, cyanide and zinc as suitable salts to form zincate and complex zinc cyanide ions, polyvinyl-alcohol or acetyl derivatives thereof, and if desired, salts of metals of the Groups VII B and VIII of the Periodic System, and a monosaccharide or polysaccharide, as they are present in the known bright zinc electroplating baths, a reaction product of

- a. a polyalkylene imine such as polyethylene imine or 65 polypropylene imine with
- b. an aromatic aldehyde,
- c. ammonia and/or ethylenediamine and diethylene triamine respectively, and

d. epichlorohydrin. Said reaction product is prepared by first reacting components (a) and (b) in an aqueous medium, such as water at a temperature between 20°C. and 50°C., adding component (c) and subsequently adding component (d) and heating the reaction mixture to a temperature of between 30°C. and 60°C., if desired, with further dilution of the reaction mixture with water. The solution of the reaction product obtained may be used without separating the reaction product. The amounts of said reaction product (calculated as non-aqueous product) added to the zinc plating bath are between 0.1 g./l. and 10 g./l., preferably between 0.2 g./l. and 5.0 g./l. of zinc bath. The amounts of zinc are normally between 5 g./l. and 50 g./l. and the amounts of cyanide are between 5 g./l. and 160 g./l. of zinc bath. Such a bath has an alkali metal cyanide: Zinc ratio (M-factor) between 1 and 3.2.

As aromatic aldehydes, there are preferably used benzaldehydes, halogen- or hydroxyl-substituted benzaldehydes such as 2,4-dichlorobenzaldehyde, p-hydroxy benzaldehyde, and other aldehydes of the general formula



In said formula

R indicates hydroxyl and/or lower alkoxy with 1 to 4 carbon atoms and especially methoxy, while

X indicates one of the numerals 0, 1, or 2. Preferred aldehydes of this type are salicylaldehyde, anisaldehyde, vanillin, and veratraldehyde.

The molecular proportions of the components of the 40 brightening reaction product added to the zinc plating bath are preferably as follows:

Molecular proportion of polyethylene imine or respectively, polypropylene imine to aromatic aldehyde between about 1 : 1 and 1 : 15;

molecular proportion of polyethylene imine or, respectively, polypropylene imine to epichlorohydrin = between about 1 : 3 and about 1 : 40;

molecular proportion of ammonia or, respectively, ethylene diamine or diethylene triamine to epichlorohydrin = 1 : 1.

Salts of manganese or nickel are preferably used as salts of a metal of the Groups VIIB or VIII of the Periodic System. They are employed in amounts between 0.01 g./l. and 0.1 g./l. and preferably between 0.01 g./l. and 0.05 g./l.

Polyvinylalcohol or an acetyl derivative thereof having a degree of polymerisation between about 300 and about 1500, such as sold under the tradename Mowiol by Farbwerke Hoechst is added in an amount between 0.05 g./l. and 0.5 g./l. and preferably in an amount between 0.1 g./l. and 0.5 g./l.

As mono- and polysaccharides one or several of dextrose, glucose, saccharose and dextrines are preferably added in an amount between 0.01 g./l. and 0.08 g./l.

## DESCRIPTION OF THE PREFERRED EMBODIMENTS

The following examples serve to illustrate the present invention without, however, limiting the same thereto.

## EXAMPLE 1

Smooth and even, bright zinc deposits on iron are obtained with a bath of the following composition, said bath having excellent throwing power, metal distribution, and brilliance. The amounts of its components are given as amounts in grams per liter of bath:

|                               |       |
|-------------------------------|-------|
| Zinc calculated as zinc oxide | 7 g.  |
| Sodium cyanide                | 10 g. |
| Sodium hydroxide              | 80 g. |

5

## Reaction product of

- polyethylene imine,
- veratraldehyde,
- ammonia, and
- epichlorohydrin

in the following proportions:

(a) : (b) = 1:1 moles;  
 (a) : (d) = 1:3 moles;  
 (c) : (d) = 1:1 moles

|                                   |                   |
|-----------------------------------|-------------------|
| Polyvinylalcohol (Mowiol N-30-88) | 0.2 g. to 5.0 g.  |
| Dextrose                          | 0.05 g. to 0.5 g. |
| Manganese sulfate                 | 0.5 g. to 5.0 g.  |
| Nickel sulfate                    | 0.02 g.           |

|  |         |
|--|---------|
|  | 0.06 g. |
|--|---------|

10

Such a bath is used at a bath temperature between 15°C. and 35°C.

The current density is between 0.3 amp./sq.dm. and 5.0 Amp./sq./dm.

15

Polyethylene imine can be replaced in said example by the equivalent amount of polypropylene imine.

In place of ethylene diamine, there can also be used 40 cc. of a 36% ammonia solution.

The benzaldehyde can be replaced by equimolecular amounts of other aromatic aldehydes.

I claim:

1. In an alkaline zinc electroplating bath comprising, in aqueous solution, a zinc salt, an alkali metal cyanide, an alkali metal hydroxide, and a water-soluble polyvinylalcohol, the improvement which comprises said bath containing, as brightening agent, between about 0.1 g./l. and about 10.0 g./l. of the reaction product obtained by reacting in an aqueous medium at a temperature between about 20° and 50°C.

- a polyalkylene imine selected from the group consisting of polyethylene imine and polypropylene imine, with
- an aromatic aldehyde, in a molar ratio between about 1:1 to 1:50 of imine to aldehyde, adding
- a basic agent selected from the group consisting of ammonia, ethylene diamine, and diethylene triamine, and
- epichlorohydrin, in a molar ratio between about 1:3 to 1:40 of imine to epichlorohydrin and about 1:1 of basic agent to epichlorohydrin, and heating the reaction mixture.

2. The zinc electroplating bath of claim 1 additionally containing a salt of a metal selected from the group consisting of a metal of the Groups VIIB and VIII of the Periodic System.

3. The alkaline zinc electroplating bath of claim 2, wherein said metal salt is present in an amount of between about 0.01 and 0.1 g./l.

4. The zinc electroplating bath of claim 1 additionally containing a mono- or polysaccharide.

5. The alkaline zinc electroplating bath of claim 3, wherein said mono- or poly-saccharide is present in an amount of between about 0.01 and 0.08 g./l.

6. The zinc electroplating bath of claim 1 additionally containing a salt of a metal selected from the group consisting of a metal of the groups VIIB and VIII of the Periodic System and a mono- or polysaccharide.

7. The alkaline zinc electroplating bath of claim 6, wherein said metal salt is present in an amount of between about 0.01 and 0.1 g./l. and said mono- or poly-saccharide is present in an amount between about 0.01 and 0.08 g./l.

8. The zinc electroplating bath of claim 1, in which the aromatic aldehyde component of the reaction product is an aromatic aldehyde selected from the group consisting of benzaldehyde, a halogen-substituted

|                                 |               |
|---------------------------------|---------------|
| Zinc (calculated as zinc oxide) | 7 g. to 30 g. |
| Sodium cyanide.                 | 81.5 g.       |
| Sodium hydroxide.               | 95 g.         |

40

Reaction product made from  
 Zinc (calculated as zinc oxide)  
 Sodium cyanide.  
 Sodium hydroxide.

Reaction product made from

Reaction product made from  
 a. polypropylene imine,  
 b. benzaldehyde,  
 c. ethylenediamine, and  
 d. epichlorohydrin  
 in the following proportion:

|                                   |                   |
|-----------------------------------|-------------------|
| (a) : (b) = 1:1 moles;            | 0.2 g. to 5.0 g.  |
| (a) : (d) = 1:10 moles;           | 0.5 g. to 5.0 g.  |
| (c) : (d) = 1:1 moles             | 0.02 g.           |
| Glucose.                          | 0.05 g.           |
| Manganese sulfate.                | 0.05 g.           |
| Nickel sulfate.                   | 0.05 g.           |
| Polyvinylalcohol (Mowiol N-30-98) | 0.05 g. to 0.5 g. |

45

Such a bath is used at a bath temperature between 15°C. and 35°C.

The current density is between 0.3 Amp./sq.dm and 5.0 Amp./sq. dm.

50

## EXAMPLE 3

The reaction product of the polyalkylene imine, an aromatic aldehyde, ethylene diamine and/or ammonia, and epichlorohydrin is prepared as follows:

25 g. (0.01 mole) of polyethylene imine are reacted

55

60

65

benzaldehyde, a hydroxyl-substituted benzaldehyde, and an aromatic aldehyde of the formula



in which

R is a member selected from the group consisting of hydroxyl and lower alkoxy with 1 to 4 carbon

atoms and  
X is a numeral selected from the numerals of 0, 1, and 2.

5 9. The alkaline zinc electroplating bath of claim 1, in which said bath contains, as brightening agent, between about 0.2 g./l. and about 5.0 g./l of the reaction product of

- 10 a. a polyalkylene imine selected from the group consisting of polyethylene imine and polypropylene imine, with  
b. an aromatic aldehyde,  
c. a basic agent selected from the group consisting of ammonia, ethylene diamine, and diethylene triamine, and  
d. epichlorohydrin.

\* \* \* \* \*

20

25

30

35

40

45

50

55

60

65

UNITED STATES PATENT OFFICE  
CERTIFICATE OF CORRECTION

Patent No. 3,915,815 Dated October 28, 1975

Inventor(s) REINHARD KOCH

It is certified that error appears in the above-identified patent and that said Letters Patent are hereby corrected as shown below:

Column 1, line 6: "bath and more particularly" should be cancelled.

line 7: "to a" should be cancelled.

line 8: After "bath" there should be added  
-- and more particularly to a --.

Signed and Sealed this  
*tenth Day of February 1976*

[SEAL]

*Attest:*

**RUTH C. MASON**  
*Attesting Officer*

**C. MARSHALL DANN**  
*Commissioner of Patents and Trademarks*